

## UNITED STATES PATENT OFFICE

2,678,301

## METHOD OF PREPARING AN ALKALINE CONCENTRATE OF MAHOGANY SULFONATES

Lionel S. Galstaun, Oakland, Calif., assignor to Tide Water Associated Oil Company, San Francisco, Calif., a corporation of Delaware

No Drawing. Application June 8, 1951,  
Serial No. 230,681

5 Claims. (Cl. 252—33)

1

This invention relates to the manufacture of petroleum mahogany sulfonates and oil concentrates thereof for use as additives for lubricating oils. More particularly, it relates to such sulfonates possessing a high degree of alkalinity especially adapted as components of lubricating oils designed for use in diesel and high output gasoline engines.

It is the primary object of the invention to provide a convenient method of preparing oil concentrates of alkaline earth metal mahogany sulfonates possessing an increased degree of alkalinity. It is a further object to utilize such sulfonates in lubricating oil compositions of value in the lubrication of diesel engines operating on high sulfur fuels. Other objects may be apparent from the following description.

Among the many additives which have been proposed for oils designed for use in the crankcases of internal combustion engines, one of the most common types employed is the metallic salts of sulfonic acids, generally referred to as metal sulfonates. Of these, the salts of mahogany sulfonic acids derived from the sulfonation of petroleum oils have found wide usage, alone or in combination with other additives, as "detergents" in crankcase oils. Recently, with the more extended use of diesel fuels having a high sulfur content, the art has shown a preference for mahogany sulfonates which have an alkaline reaction, as these, in addition to their detergent properties, have proved helpful in counteracting the effects of acidic combustion products which find their way into the crankcase when high sulfur fuels are used. In fact, it appears desirable for the sulfonate to have as high an alkalinity as possible.

A method which has been proposed for producing alkaline mahogany sulfonates is to subject a selected petroleum oil fraction to sulfonation with concentrated or fuming acid, whereby mahogany sulfonic acids are formed dissolved in the oil. After separation of the acid sludge, the dissolved sulfonic acids are neutralized by the addition of an excess of lime or other oxide or hydroxide of an alkaline-earth metal thereby forming alkaline earth mahogany sulfonate dissolved in the oil. In order to prepare a concentrate of the sulfonate for blending into other oils, the sulfonate-containing oil is subjected to distillation with steam or vacuum in order to remove the major part of the oil. By this procedure it has been possible to produce a sulfonate concentrate having an alkalinity indicating an excess of alkaline earth metal over that theo-

2

retically required to produce a neutral sulfonate. Though not exactly known, it is thought that the excess alkalinity is caused by the presence of basic sulfonates in the product.

5 According to the present invention, I have found that, by conducting the distillation step under very high vacuum and with extremely short heating period, in the order of one minute or less, sulfonate concentrates can be prepared having an alkalinity practically double that produced with conventional vacuum or steam distillation, with corresponding increase in effectiveness when blended in diesel lube oils. I have also found that, by proper selection of stocks for the sulfonation step, the alkalinity of the final concentrate may be further increased.

While in its broader aspects the invention may be practiced by sulfonating almost any sulfonatable petroleum fraction, the preferred oil for the sulfonation step is a Mid-Continent oil fraction which has been previously refined by the well known furfural selective solvent extraction process and which has a viscosity of about 150 to 400 seconds S. U. @ 100° F. I have found that this type of stock produces greater yields of sulfonates of lower viscosity thereby permitting greater concentration without producing an unmanageable concentrate. Pretreatment of the stock by other selective solvent processes, or even by 98% H<sub>2</sub>SO<sub>4</sub>, may be found to be equivalent in some respects to the furfural refining. The base oil is sulfonated by contact with a sulfonating agent such as sulfuric acid of 98% to 108% strength. However, I prefer to use 103% fuming acid, and to apply the acid in three successive treatments of 30 pounds per barrel each, removing the acid sludge formed at each stage before the succeeding stage. A temperature range of 70° to 150° F. have been found satisfactory for each stage but 90° F. to 100° F. is preferred. The three stage treatment is to be preferred over a single stage of 90 pounds per barrel, as it is found to produce a greater yield of sulfonic acid. After three stages of 30 pounds per barrel each vary little, if any, further sulfonation will occur by further treatment with additional acid. The acid sludge from the last stage is completely removed by centrifuging, filtration, or other equivalent procedure.

50 To the acid-oil there is added lime, barium hydroxide, or other alkaline earth oxide or hydroxide in an amount at least double that theoretically required to neutralize the acidity of the oil. It has been found convenient to add the base in the form of a paste containing about 2%

free water. The mixture of oil and base is thoroughly agitated until the reaction is complete, which may take an hour or so. The reaction may be assisted, especially toward the end, by heating to a temperature not exceeding about 300° F., using pressure, if desired, to avoid volatilization of the water. After neutralization the oil is clarified by filtration, using a filter-aid if desired, to yield a solution of alkaline earth metal sulfonate in a very highly treated oil stock. The sulfonate content of the oil may be about 10%, more or less, depending upon various factors such as the stocks chosen for sulfonation and the sulfonating conditions.

Though this oil-sulfonate solution may have some commercial utility, either as a lubricant per se or diluted with other oil, the oil constituent thereof is not well suited for diesel engine lubrication due, among other things, to the fact that the oil has been too highly treated with acid and the probability that the viscosity is different from that desired. Accordingly, the oil-solution is distilled to remove the greater portion of its oil content. For the purposes of the invention such distillation is carried out in a still capable of conducting the distillation at temperatures below about 300° F. while maintaining the oil at such temperature for a maximum of one minute.

A type of still suitable for conducting such distillation is that type generally referred to as "molecular stills" by those familiar with high vacuum, short path, short heating cycle distillation. In one form of these stills oil is fed upon a heated rotating plate within an assembly which is held at a high vacuum in the order of 2 to 50 microns of mercury. During the extremely short time that the oil is in contact with the plate, vaporization occurs and the vaporized molecules impact a cooled surface adjacent to the rotating plate, the distance between the two being in the order of the mean-free path of the vaporized molecules. Another form of these stills adaptable for carrying out the invention is described in U. S. Patent Number 2,210,928 issued August 13, 1940, to K. C. D. Hickman.

From the distillation of the sulfonate-oil solution a distillate oil is recovered amounting in volume to about 75% to 80% of the charge to the still. This distillate oil is normally a light colored oil suitable for use as a technical "white" oil and may be disposed of as desired. The residue from the distillation is the desired concentrate containing roughly 50% by weight of alkaline-earth sulfonate having an alkalinity remarkably higher than that produced by conventional distillation of similarly produced sulfonate-oil solutions. The concentrate may be added in any desired amount to suitable oils for the preparation of diesel lubricants. Due to the high alkalinity of the sulfonate, diesel lubricating oils prepared with the concentrate exhibit a great effectiveness in nullifying the detrimental effects which sulfur containing fuels have on the lubricating oil.

The following examples illustrate the great improvement resulting from low temperature, practically instantaneous distillation compared with conventional distillation.

#### EXAMPLE I

Ten gallons of neutral oil manufactured by furfural solvent extraction, solvent dewaxing, and final clay treatment, and having the properties shown in Table I, were sulfonated at 90° F.

with a total of 90 pounds of 103% fuming sulfuric acid per barrel of the oil.

Table I

|                                   |      |
|-----------------------------------|------|
| 5 Gravity, °API                   | 30.1 |
| Flash, Cl. O. C. °F.              | 435  |
| Viscosity, second S. U. @ 100° F. | 210  |
| Viscosity index                   | 95   |
| Color, ASTM                       | 2+   |

10 The fuming acid was applied in three treatments of 30 #/bbl. each, and sludge separated from the oil at each stage. After the sludge from the last stage was separated, the acid oil was centrifuged to remove the last traces of sludge.

15 The acid oil was then titrated to determine its acidity and neutralized at room temperature, using double the indicated number of equivalents of barium hydroxide. The hydroxide was added to the acid oil in the form of a paste of the octahydrate containing about 2 percent of uncombined water. The mixture was stirred cold for one hour, then transferred to a pressure vessel equipped with a power mixer and the reaction completed at 300° F. During this step the pressure rose to between 30 and 40 p. s. i. When reaction was complete, the heating was stopped and the water driven off by releasing the pressure.

20 The dehydrated sulfonate stock was then mixed with a filter-aid (Johns Manville Hi-flow Super-cel) at a rate of 1/2 lb. filter aid per gallon of sulfonate stock. After thorough mixing, the sulfonate stock was filtered in a filter press. Yield at this stage was 6.5 gallons of sulfonate stock comprising sulfonate dissolved in highly treated oil.

25 A portion of the filtered sulfonate stock was then charged to a molecular still operated at an absolute pressure of 12 microns of mercury at a temperature of 290° F. The overhead distillate amounted to 80.3%, and the residue 19.7%, by volume of the charge to the still. The properties of the residue, or concentrate, are shown in Table II.

#### EXAMPLE II

30 A second portion of the filtered sulfonate stock was charged to a steam still and distilled until 75% of the still charge was recovered as distillate. Further concentration in the steam still was impractical because the steam distillation was terminated when the temperature of the oil reached 650° F. A concentrate amounting to 25% by volume of the still charge was recovered and its properties are compared in Table II with those of the concentrate derived from Example I.

Table II

|                                          | Sulfonate Stock Before Dist. | Residue from Example I | Residue from Example II |
|------------------------------------------|------------------------------|------------------------|-------------------------|
| Yield, percent                           | 100                          | 19.7                   | 25                      |
| Gravity, °API                            | 23.3                         | 3.8                    | 8.1                     |
| Viscosity, SSU @ 100° F.                 | 232                          | 1698                   | 1290                    |
| Viscosity, SSU @ 210° F.                 | 49.3                         | 131.7                  | 113                     |
| Ash (as sulfate) percent                 | 5.8                          | 19.3                   | 15.3                    |
| Calc. Sulfonate Content Approx., percent | 10                           | 50                     | 40                      |
| Alkalinity (as mg. KOH per gm.)          | 9.62                         | 27.7                   | 13.62                   |

70 It will be noted from Table II that the concentrate prepared in Example I possessed a remarkably higher alkalinity than that of Example II even after allowance is made for the increased concentration which was obtainable in Example I.

**5**  
**EXAMPLE III**

The processing steps of Example I were repeated using, for the oil to be sulfonated, a furfural solvent refined, solvent dewaxed and clay finished East Texas oil of the following properties:

|                         |       |
|-------------------------|-------|
| Gravity, ° API          | 29.1  |
| Viscosity, SSU @ 100° F | 450   |
| Viscosity, index        | 94    |
| Color, ASTM             | 1 1/4 |
| Pour point ° F          | 20/25 |

The results obtained are shown in Table III.

*Table III*

|                                          | Sulfonate Stock Before Dist. | Residue from Dist. Example III |
|------------------------------------------|------------------------------|--------------------------------|
| Yield, percent                           | 100                          | 17.4                           |
| Gravity, ° API                           | 23.5                         | 4.2                            |
| Viscosity, SSU @ 100° F                  | 516                          | 4572                           |
| Viscosity, SSU @ 210° F                  | 66.4                         | 261                            |
| Ash (as sulfate) percent                 | 4.94                         | 18.5                           |
| Calc. Sulfonate Content Approx., percent | 8.5                          | 50                             |
| Alkalinity (as mg. KOH per gm.)          | 8.64                         | 30.4                           |

In the examples above barium hydroxide was used to neutralize the sulfonic acids. Calcium and strontium hydroxides may also be used. With the use of calcium hydroxide, it is occasionally found that the calcium sulfonate concentrate is very viscous and, consequently, difficult to handle. In such cases the use of one equivalent of calcium hydroxide followed by an equivalent of barium hydroxide will generally result in sulfonate concentrates having desired high alkalinity and relatively low viscosity. Thus, in a specific embodiment, the invention contemplates the use of two or more alkaline earth metal hydroxides in combination.

Concentrates prepared as described above may be blended in various percentages in petroleum lubricating oils of suitable grade for diesel lubrication. The higher alkalinity resulting from distillation in stills of the "molecular" type permits the use of less concentrate to provide the same protection against high sulfur fuels, or, with the same percent of added sulfonate, substantially greater protection against the high sulfur fuels is obtained. Ordinarily, percentages of the concentrate ranging from about 1% to about 6%, giving a sulfated ash content to the finished oil of about 0.2% to about 1.2%, have been found most useful though, in its broadest aspects, the invention is not limited by the specific values. In fact, under extremely severe diesel service, even larger amounts, such as 10% of concentrate, or even higher are of practical advantage. As is obvious, other additives may be added to the oil for other purposes, such as for example, corrosion and oxidation inhibitors, pour point depressors, and the like. Likewise, the concentrates of this invention may be used in combination with other detergents. As an example, the highly alkaline concentrate of the invention has been found to be very satisfactory for use in conjunction with calcium phenate, especially in the proportion of about 2 parts concentrate to about 2 to 3 parts calcium phenate.

As an example of a finished diesel lubricating oil prepared according to the invention, to a solvent refined Mid-Continent oil having a viscosity of 65 S. S. U. @ 210° F. and a viscosity index of 95 there is added a concentrate similar to that described in Example I and also an oxidation or

**6**  
bearing corrosion inhibitor comprising zinc alkyl thiophosphate in the following proportions:

|                       |      |
|-----------------------|------|
| Mineral oil, per cent | 93.4 |
| Concentrate, per cent | 6.0  |
| Inhibitor, per cent   | 0.6  |
|                       | 100  |

Since the concentrate, inhibitor and oil are all liquid the blending is readily done by simple mixing, using some heat to reduce the viscosity of the components and/or mixture. The resulting oil, containing about 3% sulfonate of high alkalinity, although substantial improvement can be found even at 1% sulfonate, is well suited for the lubrication of diesel engines, especially those operating on high sulfur fuels, although it is also of utility in other applications, such as gasoline fueled engines where conditions are normally unfavorable to oil stability.

I claim:

1. The method of preparing an alkaline concentrate of mahogany sulfonates useful as diesel lubricating oil component, which comprises: sulfonating a petroleum oil with a sulfonating agent to produce mahogany sulfonic acids dissolved in oil, removing the spent sulfonating agent, treating the oil containing sulfonic acids with an alkaline earth metal base in amount at least double that required theoretically to neutralize said acids thereby converting said acids to alkaline earth metal sulfonates dissolved in the oil, and distilling the thus neutralized oil at a temperature of not over about 300° F., at a pressure not exceeding 50 microns of mercury and with a heating cycle of not over one minute to remove the major part of the oil content as distillate and leave as residue an alkaline reacting concentrate of sulfonates dissolved in oil.
2. The method of claim 1 in which the petroleum oil is a refined Mid-Continent oil fraction having a Saybolt Universal viscosity at 100° F. between 150 and 400 seconds.
3. The method of claim 1 in which the alkaline earth metal base is a member of the group consisting of calcium oxide, calcium hydroxide, and barium hydroxide.
4. The method of claim 1 in which the oil containing sulfonic acids is treated with approximately one equivalent of calcium hydroxide and then with at least one equivalent of barium hydroxide thereby converting said acids to relatively low viscosity sulfonates dissolved in the oil.
5. In the concentration of alkaline reacting alkaline earth metal mahogany sulfonates dissolved in a viscous oil, the improvement which comprises distilling off excess oil from the sulfonate-oil solution at a temperature below about 300° F., at a pressure below 50 microns of mercury, and with a heating cycle not exceeding about 1 minute, whereby the sulfonate concentrates thus produced have a greatly increased alkalinity over that which would be obtained by conventional vacuum or steam distillation.

References Cited in the file of this patent

UNITED STATES PATENTS

| Number       | Name          | Date          |
|--------------|---------------|---------------|
| 70 2,229,209 | Houghton      | Jan. 21, 1941 |
| 2,402,325    | Griesinger    | June 18, 1946 |
| 2,467,176    | Zimmer et al. | Apr. 12, 1949 |
| 2,485,861    | Campbell      | Oct. 25, 1949 |
| 2,501,731    | Mertes        | Mar. 28, 1950 |
| 2,617,049    | Asseff        | Nov. 4, 1952  |